

## UNITED STATES PATENT OFFICE

2,100,408

FINISH FOR FABRICS OF ORGANIC DERIVA-  
TIVES OF CELLULOSEHerbert Platt, Cumberland, Md., assignor to  
Celanese Corporation of America, a corporation  
of DelawareNo Drawing. Application June 18, 1935,  
Serial No. 27,178

12 Claims.

(Cl. 91—68) 117-64

This invention relates to the finishing of textile material made of or containing organic derivatives of cellulose and more specifically to the finishing of fabrics to impart smoothness thereto, 5 to prevent slipping of the weave or stitch shape and to otherwise enhance its properties.

An object of the invention is the production of a sized fabric having a desired hand. Another object of the invention is the sizing of a fabric 10 to produce a smooth, soft hand with or without a delustering of the material. Another object of the invention is the anchoring of the weave or stitch shape of a fabric to prevent the same from slipping or becoming distorted and thereby producing undesired moire or other effects. Other 15 objects of the invention will appear from the following detailed description.

Sizes have been employed on textile materials containing cotton, regenerated cellulose, silk 20 and/or wool to produce a soft, non-slipping fabric. I have now found that sizes may be applied, in accordance with this invention, to textile materials containing filaments or fibres of artificial materials, such as the organic derivatives of cellulose. The physical and chemical nature of 25 filaments and fibres containing organic derivatives of cellulose is such that sizes and processes of sizing normally employed in the textile art are not applicable thereto. Many of the sizes formerly employed would not sufficiently adhere to 30 or penetrate into textile materials containing a substantial amount of filaments or fibres of organic derivatives of cellulose, to produce a non-slipping fabric, while other sizes make the fabric stiff, harsh or otherwise deleteriously modify the 35 hand of the fabric. Fabrics containing organic derivatives of cellulose that have a size applied thereto in accordance with my invention have a full or weighted but soft hand and may be produced with a natural or subdued luster.

In accordance with my invention, I apply to fabrics containing organic derivatives of cellulose a solution or suspension of the resulting product formed by mixing together a resin, ammonia 45 and sodium silicate in water and alcohol. The fabric is preferably pre-dyed, rinsed free from soap and oil and vacuum extracted on the jig prior to treatment with the sizing solution or suspension. The sizing material is preferably placed upon the fabric and the fabric immediately passed through a tenter where it is dried with practically no tension crosswise the fabric. If a delustered appearance is desired, the fabric 55 may be treated, after sizing, with a solution of

a salt that reacts with the material of the sizing to form substantially insoluble resinate.

This invention is applicable to fabrics made of or containing filaments or fibres of organic derivatives of cellulose. The filaments or fibres containing organic derivatives of cellulose may be made from one or a mixture of any suitable organic ester of cellulose or cellulose ether. Examples of organic esters of cellulose are cellulose acetate, cellulose formate, cellulose propionate and cellulose butyrate, while examples of cellulose ethers are ethyl cellulose, methyl cellulose and benzyl cellulose.

The fabric may consist wholly of yarns consisting of fibres or filaments of organic derivatives of cellulose or the yarns may contain, in addition to organic derivatives of cellulose fibres and filaments, other textile materials such as fibres or filaments of cotton, wool, regenerated cellulose, silk, etc. Further, the fabric may be formed from yarns consisting of organic derivatives of cellulose interwoven or interknitted in any suitable manner with yarns formed of other textile materials or mixtures of textile materials.

The fabric may be formed by weaving, circular knitting, warp knitting or netting the yarn. The invention is of particular importance, however, to the treatment of fabrics woven with a taffeta or similar weave. However, the invention is also of importance in the treatment of circular knit material to lend to the same a weighted but soft hand.

The sizing material or finishing material may be formed by mixing together any suitable resin or resinous material and alcohol. When the solution of resin and alcohol is almost complete a suitable quantity of ammonia or other basic material may be added. The solution of resin and ammonia or the chemical reaction products of the same may then be strained or filtered free of solids or foreign materials. This mixture forms the stock solution of the sizing material. The sizing material or the solution or suspension that is padded upon the textile fabric may be formed from the above stock solution by diluting the same with water and adding thereto sodium silicate.

The textile material after being rinsed free from soap and oil and vacuum extracted may be treated with the size by immersing the fabric in the sizing bath and passing the same between nip rollers. The fabric preferably passes directly from the nip rollers to a tenter where it is dried with as low a tension as possible. After the material has passed through a tenter, it is pref-

106. COMPOSITIONS,  
COATING OR PLASTIC.

83

2,100,408

erable to give it one, two or more passes between heated nip rollers of a hot calender, the rolls of which are maintained at between 95° C. and 115° C.

5 For the purpose of illustrating the invention and not as a limitation, the following preferred example is given:

## EXAMPLE

10 A stock solution of ammonia and resin

|                    | Parts by volume |
|--------------------|-----------------|
| Resin              | 463             |
| Ethyl alcohol      | 1000            |
| Ammonium hydroxide | 250             |
| 15 Water           | 8287            |

The resin and alcohol are mixed together and when the solution is almost complete the ammonia may be added. The mixture then may be 20 allowed to stand with occasional stirring until practically all of it is in solution. The solution then may be filtered to remove solid materials and foreign matter. The solution so produced may be diluted to 10,000 parts by volume with 25 water to form a stock solution for sizing purposes.

To the stock solution may be added a solution of sodium silicate sufficient to make the strength of the sodium silicate in the resulting 30 solution 5 grams per litre. The sodium silicate preferably is added to the stock solution just prior to the employment of the solution. This solution is then padded onto a fabric containing organic derivatives of cellulose in the manner described 35 above.

Any suitable resin or resinous material may be employed, it being preferable, however, to employ a bleached natural resin. Such other resins may be employed as the commercial or brown 40 natural resin, and synthetic resins that are soluble in alcohol or similar solvents and that form substantially insoluble salts with barium. The resin or resinous material employed should be soluble in alcohol or similar solvent. The amount 45 of resin employed may vary from that given in the example. For instance, one may employ from 400 to 800 parts by volume to every 10,000 parts by volume of stock solution formed.

Any suitable alcohol may be employed in forming 50 the stock solution. It is preferable, however, to employ commercial grades of ethyl alcohol. Other alcohol such as methyl alcohol, denatured ethyl alcohol or butyl alcohol may be substituted for all or a part of the commercial ethyl alcohol. Solvents other than alcohol may be employed and their use and nature will depend upon 55 the resinous substance employed. The amount of alcohol or solvent employed may vary from the amount stated in the example. Depending 60 somewhat upon the resin employed, the quantity of alcohol or resin solvent employed may vary from 500 to 2000 parts by volume.

Ammonium hydroxide is the preferred alkaline 65 material to be added to the resin. However, other basic materials may be employed, for instance sodium or potassium hydroxide. The quantity of basic material employed may vary from the quantity recited in the example and may be from 200 to 350 or more parts by volume to each 10,000 70 parts of stock solution produced.

If it is desired to form a subdued lustre on the material, the same may be given after a dip and a nip through the resin-silicate solution or suspension, a further padding in a barium chloride 75 or similar salt solution. The solution may con-

tain from 5 to 20% or more of barium chloride dissolved in water. It is preferred, however, to employ a 10% solution of barium chloride. The padding operation is preferably done by passing the material, treated with the resin size, through 5 the solution containing barium chloride or other salt and twice through nip rollers on a cold calender. Although barium chloride is preferred, other salts that will react with the resinous material to form substantially insoluble salts may be 10 employed. Examples of such salts are calcium chloride, strontium chloride or other soluble halogen salts of the same or similar metals. The fabric may be padded with the resin-silicate, then with or without drying it may be padded with 15 the salt solution.

It is understood that the foregoing detailed description is given merely by way of illustration and that many variations may be made therein without departing from the spirit of my invention. 20

Having described my invention, what I desire to secure by Letters Patent is:

1. In a method of finishing fabrics containing 25 derivatives of cellulose containing organic substituent groups to impart thereto a smooth hand and prevent slipping of weave and stitch distortion, the step of applying to the fabric a liquid medium comprising the resultant product obtained by mixing together in a liquid a resinous 30 material, an alkaline material and sodium silicate.

2. In a method of finishing fabrics containing cellulose acetate to impart thereto a smooth hand and prevent slipping of weave and stitch distortion, the step of applying to the fabric a liquid medium comprising the resultant product obtained by mixing together in a liquid a resinous 35 material, an alkaline material and sodium silicate.

3. In a method of finishing fabrics containing derivatives of cellulose containing organic substituent groups to impart thereto a smooth hand and prevent slipping of weave and stitch distortion, the step of padding the fabric with a 45 liquid medium comprising the resultant product formed by mixing together a natural resin, an alkaline material and sodium silicate in a liquid.

4. In a method of finishing fabrics containing cellulose acetate to impart thereto a smooth hand 50 and prevent slipping of weave and stitch distortion, the step of padding the fabric with a liquid medium comprising the resultant product formed by mixing together natural resin, an alkaline material and sodium silicate in a liquid. 55

5. In a method of finishing fabrics containing cellulose acetate to impart thereto a smooth hand and prevent slipping of weave and stitch distortion, the step of padding the fabric with a liquid medium comprising the resultant product formed 60 by mixing together natural resin, ammonium hydroxide and sodium silicate in a liquid.

6. In a method of finishing fabrics containing cellulose acetate to impart thereto a smooth hand and prevent slipping of weave and stitch distortion, the step of padding the fabric with a liquid medium comprising the resultant product formed 65 by mixing together bleached natural resin, ammonium hydroxide and sodium silicate in a liquid.

7. In a method of finishing fabrics containing derivatives of cellulose containing organic substituent groups to impart thereto a smooth hand and prevent slipping of weave and stitch distortion, the step of padding the fabric with a liquid medium formed by mixing together from 400 to 70 75

- 800 parts by volume of a resin, from 500 to 2,000 parts by volume of ethyl alcohol, from 200 to 350 parts by volume of ammonium hydroxide, and sufficient water to make 10,000 parts of solution, and adding sufficient sodium silicate to give a concentration of 5 grams of sodium silicate per litre of solution.
8. In a method of finishing fabrics containing derivatives of cellulose containing organic substituent groups to impart thereto a smooth hand and prevent slipping of weave and stitch distortion, the steps of applying to the fabric a liquid medium comprising the resultant product obtained by mixing together in a liquid a natural resin, an alkaline material, and sodium silicate and applying to the fabric thus treated a solution of a halogen salt of an alkaline earth metal.
9. In a method of finishing fabrics containing derivatives of cellulose containing organic substituent groups to impart thereto a smooth hand and prevent slipping of weave and stitch distortion, the steps of padding the fabric with a liquid medium comprising a product formed by mixing together in a liquid a natural resin, ammonia and sodium silicate and then padding the fabric with a solution containing barium chloride.
10. A fabric containing filaments or fibers of derivatives of cellulose containing organic substituent groups having a coating thereon comprising the reaction product, formed by applying to the fabric the product formed by mixing together in a liquid carrier a natural resin, ammonium hydroxide, and sodium silicate and reacting this product with barium chloride in situ. 5
11. Fabrics comprising yarns of derivatives of cellulose containing organic substituent groups, in which the yarns are caused to adhere one to another by a coating applied to the fabric and comprising the reaction product formed by mixing together in a liquid carrier a resin, ammonium hydroxide and sodium silicate. 10
12. Fabrics comprising yarns of derivatives of cellulose containing organic substituent groups, in which the yarns are caused to adhere one to another by a coating applied to the fabric and comprising the reaction product formed by mixing together in a liquid carrier a natural resin, ammonium hydroxide and sodium silicate and reacting this composition with barium chloride. 15

HERBERT PLATT. 25